

May 2, 1967

E. C. REICHERT ET AL

3,317,365

NON-FLAMMABLE SYNTHETIC DECORATIVE TREE BRANCH

Filed June 30, 1964

3 Sheets-Sheet 1



FIG.-1

INVENTORS

ERWIN C. REICHERT  
JOHN C. LEWIS, JR.

BY

MORGAN, FINNEGAN, DURHAM & PINE

ATTORNEYS

May 2, 1967

E. C. REICHERT ET AL

3,317,365

NON-FLAMMABLE SYNTHETIC DECORATIVE TREE BRANCH

Filed June 30, 1964

3 Sheets-Sheet 2



FIG.-2

INVENTORS  
ERWIN C. REICHERT  
JOHN C. LEWIS, JR.

BY

MORGAN, FINNEGAN, DURHAM & PINE

ATTORNEYS

May 2, 1967

E. C. REICHERT ET AL

3,317,365

NON-FLAMMABLE SYNTHETIC DECORATIVE TREE BRANCH

Filed June 30, 1964

3 Sheets-Sheet 3

FIG.-3



FIG.-4



INVENTORS  
ERWIN C. REICHERT  
JOHN C. LEWIS, JR.

BY

MORGAN, FINNEGAN, DURHAM & PINE

ATTORNEYS

## 1

3,317,365

NON-FLAMMABLE SYNTHETIC DECORATIVE  
TREE BRANCH

Erwin C. Reichert and John C. Lewis, Jr., Middlebury, Vt., assignors to Polymers, Inc., Middlebury, Vt., a corporation of Vermont

Filed June 30, 1964, Ser. No. 379,087  
2 Claims. (Cl. 161—22)

This invention relates to a novel twisted-in-wire brush construction comprising a mixture of at least two synthetic fibres. The brush construction of this invention is of non-flammable nature and is particularly useful as a decorative or novelty item.

Prior to this invention, there have been employed natural and/or synthetic fibre mixtures in the manufacture of brushes, brooms and the like. In such constructions, the physical properties of the fibre mixture which generally are of importance are with respect to stiffness, tensile strength, wear qualities, abrasive qualities and fatigue resistance. Normally the fire rating or non-flammable quality is not a criterion in evaluating the suitability of a particular fibre mixture in the manufacture of articles of the above-mentioned type.

The invention is concerned with the utilization of a fibre mixture in which the fire rating or non-flammable quality of the mixture is of paramount importance since the chief use of the brush construction of this invention is for decorative purposes, particularly for synthetic Christmas tree branches where non-flammability is an essential characteristic.

In producing a brush construction of the type mentioned above, other factors must be considered in addition to the non-flammable quality of the fibre mixture. For example, it is well known that halogen-bearing fibres have non-flammable characteristics. Examples of these fibres are polyvinyl chloride, polyvinyl chloride-polycarbonate copolymers and vinylidene chloride-vinyl chloride copolymers. However, economics and the bulk density factor of round halogen-bearing fibres make it such that their usage becomes limited in manufactured items when the fibre is only used for decorative purposes and not for mechanical functions as in the case of the heretofore mentioned synthetic Christmas tree branches. In such branches, the fibres are only held by wire in space to simulate a tree branch. The only pre-requisite other than economic feasibility is that the fibres do not burn or spontaneously ignite themselves.

Objects and advantages of the invention will be set forth in part hereinafter and in part will be obvious from, or may be learned by practice with the invention, the same being realized and attained by means of the steps, methods, composition, combination and improvement pointed out in the appended claims.

This invention consists in the novel steps, methods, compositions, combinations and improvements herein shown and described.

It is an object of this invention to provide a novel brush construction which has non-flammable qualities and is sufficiently inexpensive to be useful as a decorative or novelty item.

Another object of this invention is to provide a novel twisted-in-wire brush construction which exhibits non-flammable qualities and is particularly useful as a synthetic Christmas tree branch.

In the drawings:

FIGURE 1 is a perspective view of a parallel group of cut mixed fibres used in the production of the brush construction of this invention.

FIGURE 2 is a view in perspective of the brush construction of this invention.

FIGURE 3 is a fragmentary perspective view of a

## 2

section of the brush construction of FIGURE 2 before heat or flame is applied.

FIGURE 4 is a perspective view of FIGURE 3 after heat and flame is applied.

In general practice, fibre mixtures have been limited in use because of costs involved in mixing. However, it becomes necessary to use fibre mixtures when trying to adjust a physical and/or chemical property for a given fibre (or fibres), and stay within specified and defined limits. In the case of non-flammable fibres such as vinyl chloride polymer and copolymer compositions, (containing at least 50% by weight chlorine in the molecule), it has been found that the chlorine in the chemical make-up of the molecule is what imparts the non-flammable characteristics. For convenience sake, the term "vinyl chloride polymer" as used hereinafter means both the homopolymers and copolymers (e.g. vinyl chloride-vinylidene copolymer copolymers known as "Saran" polymers). The polymer must contain at least about 50% chlorine linkage in order to make it flame retardant. But as the chlorine percent goes up, so does the specific gravity of the polymer, thus forcing the ratio of cubic inches of fibre per pound to decrease.

0.018" diameter vinyl chloride fibre has a bulk density of 24-27 cubic inches per pound. The bulk density of a mixture of vinyl chloride fibres may be increased, while still maintaining the non-flammability characteristics thereof, by combining therewith, other fibre whose specific gravity is less than that of 1.4, such, for example, as effected by adding polystyrene and/or other types of fibres to the vinyl chloride mixture. Thus if 25% by volume vinyl chloride fibre is mixed with 75% by volume styrene fibre, the bulk density is increased from 24-27 units for pure vinyl chloride to 30-31 units for the mixture of vinyl chloride and styrene and yet no significant sacrifice has to be made with respect to the non-flammability characteristics of the mixture. When the fibre mixture is twisted-in-wire to form a brush construction for use in decorative items it will not burn.

It can be shown that as the volume percent of styrene increases over 75% of the mixture, that the non-flammability characteristic decreases until the twisted-in-wire brush construction supports combustion. As will be readily apparent from the results reported in Table 3 given hereinafter, in order to achieve the desired non-flammable qualities for the fibre mixture, the vinyl chloride fibre should be in an amount at least 10% by volume of the fibre mixture.

Referring more specifically to the drawings:

In FIGURE 1 is shown the mixed fibre bundle 1 containing two different synthetic fibres, vinyl chloride (at least 50% by weight chlorine) fibre 2 and polystyrene fibre 3. It will be appreciated that if these fibres 2 and 3 are not evenly distributed in the bundle, that subsequent processing in wire sections would give concentrated areas of one type of fibre and not the other. This would destroy the non-flammability characteristics since any concentrated area of styrene would be enough to burn and render the vinyl fibre portion ineffective in eliminating the flammable characteristics.

As shown in FIGURE 2, the fibres 2 and 3 are twisted-in-wire 4 to form a section of branch for decorative uses. If the fibre mixture making up the section is properly mixed, then the twisted section also has an even distribution of the two fibres.

Reference is now made to FIGURES 3 and 4 in order to illustrate how the vinyl chloride in the vinyl chloride-styrene mixture controls the flammability of the mixture. The explanation of burning is as follows: Vinyl PVC fibre will not burn. The fibres only char and emit chloride fumes. This emission of fumes (non-combustible mixture of gases) from the decomposing vinyl causes the exclusion

of oxygen in the air around the area of the fibre. This same principle of oxygen elimination can be applied when a mixture of fibres (i.e. vinyl and styrene) are burned. The vinyl cannot burn due to the chemical nature and as it decomposes, the gases deprive the styrene of oxygen. Thus the whole mass of fibre only melts and decomposes into charred carbon.

From FIGURE 3 it can be seen that as heat and fire begin to melt and char fibres 2 and 3 these fibres shrink and tend to collapse toward the center of wire frame 4. As this takes place, the fibres 2 and 3 now in FIGURE 4, are no longer in the open air. Thus, as the vinyl fibre 2 decomposed, it eliminated the oxygen from the area, and the styrene fibre 3 cannot burn.

In order to describe the invention in greater detail, the following examples are now given:

Twisted-in-wire tree branch brush construction were fabricated to the following specifications:

The sections consisted of an overall 24 inch wire with a brush face of approximately 12 inches and an overall trim of 3 inches. Where the fibre mixture of the brush construction was all vinyl chloride fibre, its weight was approximately 1 oz. Where the fibre mixture is other than all vinyl chloride, its weight is less than 1 oz. since the fibres other than vinyl chloride fibre have a higher bulk density. Brush constructions were fabricated using the following types of fibres and fibre combinations. (The wire used was regular twisting wire used in the manufacturing of twisted-in-wire sections.)

|                                         | Percent |
|-----------------------------------------|---------|
| Vinyl PVC (over 50% by weight chlorine) | 100     |
| Styrene                                 | 100     |
| Propylene                               | 100     |
| Ethylene                                | 100     |
| Vinyl PVC and styrene                   | 50/50   |
| Vinyl PVC and styrene                   | 33/66   |
| Vinyl PVC and styrene                   | 25/75   |
| Vinyl PVC and styrene                   | 20/80   |
| Vinyl PVC and styrene                   | 10/90   |
| Vinyl PVC and propylene                 | 50/50   |
| Vinyl PVC and ethylene                  | 50/50   |

Special sections were twisted using vinyl PVC-coated wire:

|           | Percent |
|-----------|---------|
| Styrene   | 100     |
| Propylene | 100     |
| Ethylene  | 100     |

The following test procedures were employed in evaluating the flammability of the above-mentioned brush constructions, the results of said tests being reported in Tables 1-3 appearing hereinafter.

(A) An individual branch section was suspended vertically from a pipe and wire over a metal dish. The bottom of the section was held approximately 4-inches from the metal dish. (The extra metal wire from the twisting operation was cut off allowing fibre to be 4-inches from the dish.)

(B) A 10 gram fire (10 grams of cut newspaper) was placed under the section. As the paper burned, the head and flames were allowed to rise vertically through the section. (The 10 gram fire had an average burning time of 40 seconds.)

(C) The paper was ignited and allowed to burn. If after the paper fire had burned out a fire started in the section, then it determined that the section supported combustion and was labeled "supports combustion." On the other hand, if after the paper fire had burned out no fire had started, but only melting and charring of the fibres took place, then the section was labeled "non-flammable."

(D) Also, a complete physical examination was carried out on each section to determine the amount of burning, melting, charring, etc.

(E) A second method of burning was carried out. A torch was placed under each section and held for two minutes.

The same classifications were given the sections after each two minute test.

The following Table I gives the results of branch sections burned using a controlled fire of 10 grams (40 second fire).

TABLE I

| Composition <sup>1</sup> | Weight, oz. | Number Inches Burned/Char | Remarks            | Rating         |
|--------------------------|-------------|---------------------------|--------------------|----------------|
| 100% Vinyl PVC           | 1           | 8-10                      | Chars <sup>2</sup> | Non-flammable. |
| 100% Styrene             | 3/4         | 12                        | Burns              | Supports Fire. |
| 100% Propylene           | 1/2         | 12                        | do                 | Do.            |
| 100% Ethylene            | 1/2         | 12                        | do                 | Do.            |
| 50/50% PVC/Styrene       | 3/4         | 8-10                      | Chars <sup>3</sup> | Non-flammable. |
| 33/66% PVC/Styrene       | 3/4         | 8-10                      | do <sup>3</sup>    | Do.            |
| 27/75% PVC/Styrene       | 3/4         | 8-10                      | do <sup>4</sup>    | Do.            |
| 20/80% PVC/Styrene       | 3/4         | 10-11                     | do <sup>4</sup>    | Do.            |
| 10/90% PVC/Styrene       | 3/4         | 10-11                     | do <sup>5</sup>    | Supports Fire. |
| 50/50% PVC/Propylene     | 1/2         | 8-10                      | do <sup>3</sup>    | Non-flammable. |
| 50/50% PVC/Ethylene      | 1/2         | 8-10                      | do <sup>3</sup>    | Do.            |

<sup>1</sup> All fibre mixtures based on percent by volume (no coated wire).

<sup>2</sup> Does not burn—gives off chloride fumes; chars.

<sup>3</sup> Starts to burn but gases given off from PVC stop the burning; melts.

<sup>4</sup> Starts to burn—sometimes burns, but usually burns out.

<sup>5</sup> Starts to burn—continues to burn; not as rapidly as 100% styrene.

The following Table II gives results of fibres burned using vinyl-coat wire. The controlled fire was 10 grams (40 second fire).

TABLE II

| Composition <sup>6</sup> | Weight, oz. | Number Inches Burned/Char | Remarks            | Rating         |
|--------------------------|-------------|---------------------------|--------------------|----------------|
| 100% Styrene             | 3/4         | 12                        | Burns <sup>7</sup> | Supports Fire. |
| 100% Propylene           | 1/2         | 12                        | do                 | Do.            |
| 100% Ethylene            | 1/2         | 12                        | do                 | Do.            |

<sup>6</sup> Used 100% fibre material and Vinyl Coated Wire.

<sup>7</sup> Sections started to burn immediately and continued until all fibres gone.

The following Table III gives the results of branch sections burned using a 2 minute fire obtained from a gas torch.

and polyethylene, said halogen-bearing fibre being present in an amount of 10% to 50% by volume of the synthetic fibre mixture.

TABLE III

| Composition <sup>8</sup>  | Weight, oz. | Number Inches Burned/Char | Remarks                      | Rating         |
|---------------------------|-------------|---------------------------|------------------------------|----------------|
| 100% Vinyl PVC-----       | 1           | 8-10                      | Chars <sup>9</sup> -----     | Non-flammable. |
| 100% Styrene-----         | 3/4         | 12                        | Burns -----                  | Supports Fire. |
| 100% Propylene-----       | 1/2         | 12                        | ----- do -----               | Do.            |
| 100% Ethylene-----        | 1/2         | 12                        | ----- do -----               | Do.            |
| 50/50% PVC/Styrene-----   | 3/4         | 8-10                      | Chars <sup>10</sup> -----    | Non-flammable. |
| 50/50% PVC/Propylene----- | 1/2         | 8-10                      | ----- do <sup>10</sup> ----- | Do.            |
| 50/50% PVC/Ethylene-----  | 1/2         | 8-10                      | ----- do <sup>10</sup> ----- | Do.            |
| 33/66% PVC/Styrene-----   | 3/8         | 8-10                      | ----- do <sup>10</sup> ----- | Do.            |
| 25/75% PVC/Styrene-----   | 5/8         | 8-10                      | ----- do <sup>10</sup> ----- | Do.            |
| 20/80% PVC/Styrene-----   | 3/4         | 10-11                     | ----- do <sup>11</sup> ----- | Do.            |
| 10/90% PVC/Styrene-----   | 3/4         | 10-11                     | ----- do <sup>12</sup> ----- | Supports Fire. |

<sup>8</sup> All fibre mixtures based on percent by volume (no coated wire).

<sup>9</sup> Does not burn—gives off chloride fumes; chars.

<sup>10</sup> Starts to burn but gases from PVC stop the burning.

<sup>11</sup> Starts to burn—sometimes burns; usually goes out.

<sup>12</sup> Starts to burn—continues to burn—not as rapidly as 100% Styrene.

On the basis of the test results reported in the foregoing Tables I to III, it can be said that only a few combinations of mixed synthetic fibre can be successfully used in obtaining non-flammable characteristics. Any combination under at least about 10% by volume vinyl fibre is not safe for use in non-flammable decorative items of manufacture.

The fibre combinations of this invention may be used to prepare improved non-flammable decorative products such as: Christmas tree branches, wreaths, flower displays, etc.

Colorants, extenders, plasticizers, catalysts and modifiers may be added to these materials as practice dictates.

The invention in its broader aspects is not limited to the specific steps, compositions, combinations and improvements described but departures may be made therefrom within the scope of the accompanying claims without departing from the principles of the invention and without sacrificing its chief advantages.

We claim:

1. A non-flammable synthetic decorative tree branch of assembled twisted-in-wire construction whose fibres simulate tree needles and consist of a mixture of two synthetic fibres one of which is a non-flammable polyvinyl chloride fibre, and the other of which is a flammable fibre selected from the group consisting of polystyrene, polypropylene

25 2. A non-flammable synthetic decorative tree branch of assembled twisted-in-wire construction, whose fibres simulate tree needles and consist of a mixture of two synthetic fibres, one of which is a non-flammable polyvinylchloride fibre, and the second of which is polystyrene fibre, said polyvinylchloride fibre being present in an amount of 30% by volume of the synthetic fibre mixture.

#### References Cited by the Examiner

##### UNITED STATES PATENTS

|    |           |        |                       |           |
|----|-----------|--------|-----------------------|-----------|
| 35 | 2,605,514 | 8/1952 | Eshenaur et al. ----- | 161—403 X |
|    | 2,683,210 | 7/1954 | Baunziger -----       | 161—23    |
|    | 2,826,846 | 3/1958 | Warren -----          | 161—24    |
|    | 3,072,512 | 1/1963 | Dalle -----           | 161—92 X  |
|    | 3,167,467 | 1/1965 | Abramson -----        | 161—24    |

##### FOREIGN PATENTS

|         |         |                |
|---------|---------|----------------|
| 7,022   | of 1914 | Great Britain. |
| 306,713 | 2/1929  | Great Britain. |
| 955,778 | 4/1964  | Great Britain. |

45 EARL M. BERGERT, Primary Examiner.

H. ANSHER, Assistant Examiner.